

## UNITED STATES PATENT OFFICE

CAMILLE DREYFUS, OF NEW YORK, N. Y., AND HERBERT PLATT, OF CUMBERLAND, MARYLAND, ASSIGNEES TO CELANESE CORPORATION OF AMERICA, A CORPORATION OF DELAWARE

## WEIGHTING FIBERS OF CELLULOSE DERIVATIVES

No Drawing.

Application filed October 24, 1925. Serial No. 64,699.

It has been found that when fibers, fabrics or similar articles formed from organic substitution derivatives of cellulose, such as cellulose esters or ethers, and more specifically 5 cellulose acetate, are treated with solutions comprising tannic acid with or without previous or subsequent treatment with other substances to fix the tannic acid, valuable results are produced without impairing the appearance or other qualities of the materials. One 10 of these results is a substantial increase in the weight and volume of the materials treated. It also renders yarns, fibers and fabrics of such materials, and particularly of cellulose 15 acetate, more resistant to heat, so that they can be ironed with a hot iron similarly to other fabrics. The inflammability thereof is also reduced and the slipping of the fabrics is lessened. Furthermore, it is found that in 20 the case of circular knitted fabrics made with cellulose acetate silk and treated in this manner, the laddering capacity of the fabric becomes much less.

The character of the invention and the 25 mode of application thereof can probably be best set forth by giving certain examples which are to be regarded merely as illustrative and not as limiting the scope of the invention.

30 *Example No. 1*

1 part of artificial silk made from cellulose acetate is treated with 30 parts of a 30% solution of tannic acid at a temperature of about 35 55° C. for three-quarters of an hour. This results in a marked increase in weight after the silk has been rinsed. If the material is treated with a tannic acid solution of this strength in the cold, there is less increase in 40 the weight. On the other hand, a treatment with a 30% solution of tannic acid for two hours with a temperature of from 80° to 85° C. results in a very marked increase in the weight of the materials.

45 *Example No. 2:*

1 part of cellulose acetate silk is treated with 30 parts of a 30% tannic acid solution at about 55° C., then rinsed off in water and then treated with 4% tartar emetic at about 35° C.

for approximately two hours. The subsequent treatment with tartar emetic results in a further increase in the weight of the silk.

55 *Example No. 3*

Cellulose acetate artificial silk is treated with a 30% tannic acid solution for two hours at about 45° to 80° C., rinsed in water and subsequently treated with 5% stannic chloride in the cold for twenty-four hours. Excellent 60 results may be obtained by treatment with 30% solution at from 45° to 55° C.

65 *Example No. 4*

Instead of the stannic chloride in the preceding example, there may be employed a 3% solution of tartar emetic in the cold for twenty-four hours.

70 *Example No. 5*

1 part of artificial silk is treated with 30 parts of a 30% stannic chloride solution for one hour at from 40° to 65° C., then rinsed off in water and treated with 30% tannic acid for one-half hour at from 55° to 80° C. The 75 increase in weight is very great with a relatively small loss on washing, but the quality of the resultant product is not quite so satisfactory in other respects.

It will be noted that tannic acid may be 80 used alone with excellent results or that it may be followed by a subsequent treatment with stannic chloride or tartar emetic, or that the materials may be treated first with stannic chloride and subsequently with tannic acid, and it will be understood that in the claims, when speaking of treatment with a solution comprising tannic acid and with a solution comprising a metal salt, such previous treatment with the metal salt followed 85 by treatment with tannic acid is likewise included. The treatment with tannic acid alone or followed by subsequent treatment appears to be preferable. The strength of the solutions may vary and the temperature may also 90 vary. These two factors have a certain relation to each other and are also related to the duration of the reaction. The lower the temperature the longer time and stronger solution necessary. In the case of tannic acid, the 95 100

temperature limits are from cold to 85° C. and preferably from 50° to 70°. The time of reaction may vary from one-half hour to two hours. When material treated with tannic acid is subjected to a subsequent treatment with stannic chloride or tartar emetic, this is carried out either in the cold or preferably at a lower temperature than the first treatment.

10 While the process is particularly adapted for cellulose acetate silk, it is not limited in its application thereto but may be applied to fibers or fabrics of other cellulose derivatives. It may also be applied to a fabric or fiber which is entirely formed of cellulose acetate or other cellulose derivatives or to a fiber or fabric which is composed partly of such cellulose compounds and partly of other materials, such as silk, etc. In the claims it is to be understood that the term material includes fabrics, fibers, or the like, and that where treatment with a solution comprising a certain substance is mentioned, it is understood that the solution may consist solely of such substance or of such substance combined with other substances. By the term "swelling agent" as used in the claims we mean a substance or solution which is mutually soluble in cellulose acetate. Thus tannic acid itself in certain concentrations is a swelling agent as are also sufficiently concentrated solutions of some metallic salts. Other well known swelling agents of organic derivatives of cellulose are formic acid, acetic acid, phenol, furfural, pyridine, metallic thiocyanates etc. In general, it is to be remembered that the invention is to be regarded as limited only by the scope of the appended claims.

We claim:

40 1. A process for the weighting of material comprising an organic substitution derivative of cellulose, which comprises treating said material with a solution which is a swelling agent for said material and contains tannic acid in such quantity and concentration as to materially exceed that required for mordanting.

50 2. A process for the weighting of material comprising an organic substitution derivative of cellulose, which comprises treating said material with a solution which is a swelling agent for said material and contains tannic acid in such quantity and concentration as to materially exceed that required for mordanting, and with another substance adapted to fix the tannic acid.

60 3. A process for the weighting of material comprising an organic substitution derivative of cellulose, which comprises treating said material with a solution which is a swelling agent for said material and contains tannic acid in such quantity and concentration as to materially exceed that required for mordanting, and with a solution comprising a metal salt adapted to fix the tannic acid.

4. A process for the weighting of material comprising an organic substitution derivative of cellulose, which comprises treating said material with a solution which is a swelling agent for said material and contains tannic acid in such quantity and concentration as to materially exceed that required for mordanting, and subsequently treating with a solution comprising a metal salt adapted to fix the tannic acid.

70 5. A process for the weighting of material comprising an organic substitution derivative of cellulose, which comprises treating said material with a solution which is a swelling agent for said material and contains tannic acid in such quantity and concentration as to materially exceed that required for mordanting, and subsequently treating with a solution comprising tartar emetic.

75 6. A process for the weighting of material comprising an organic substitution derivative of cellulose, which comprises treating said material at about 45° to 80° C. with a solution which is a swelling agent for said material and contains tannic acid in such quantity and concentration as to materially exceed that required for mordanting.

80 7. A process for the weighting of material comprising an organic substitution derivative of cellulose, which comprises treating said material at about 45° to 80° C. with a solution which is a swelling agent for said material and contains tannic acid in such quantity and concentration as to materially exceed that required for mordanting, and with another substance adapted to fix the tannic acid.

85 8. A process for the weighting of material comprising an organic substitution derivative of cellulose, which comprises treating said material at about 45° to 80° C. with a solution which is a swelling agent for said material and contains tannic acid in such quantity and concentration as to materially exceed that required for mordanting, and with a solution comprising a metal salt adapted to fix the tannic acid.

90 9. A process for the weighting of material comprising an organic substitution derivative of cellulose, which comprises treating said material at about 45° to 80° C. with a solution which is a swelling agent for said material and contains tannic acid in such quantity and concentration as to materially exceed that required for mordanting, and subsequently treating with a solution comprising a metal salt adapted to fix the tannic acid.

100 10. A process for the weighting of material comprising an organic substitution derivative of cellulose, which comprises treating said material at about 45° to 80° C. with a solution which is a swelling agent for said material and contains tannic acid in such quantity and concentration as to materially

exceed that required for mordanting, and subsequently treating with a solution comprising tartar emetic.

11. A process for the weighting of material comprising an organic ester of cellulose, which comprises treating said material with a solution which is a swelling agent for said material and contains tannic acid in such quantity and concentration as to materially exceed that required for mordanting.

10      12. A process for the weighting of material comprising an organic ester of cellulose, which comprises treating said material with a solution which is a swelling agent for said material and contains tannic acid in such quantity and concentration as to materially exceed that required for mordanting, and with another substance adapted to fix the tannic acid.

20 13. A process for the weighting of material comprising an organic ester of cellulose, which comprises treating said material with a solution which is a swelling agent for said material and contains tannic acid in such 25 quantity and concentration as to materially exceed that required for mordanting, and with a solution comprising a metal salt adapted to fix the tannic acid.

14. A process for the weighting of material comprising an organic ester of cellulose, which comprises treating said material with a solution which is a swelling agent for said material and contains tannic acid in such quantity and concentration as to materially exceed that required for mordanting, and subsequently treating with a solution comprising a metal salt adapted to fix the tannic acid.

acid.

15. A process for the weighting of material comprising an organic ester of cellulose, which comprises treating said material with a solution which is a swelling agent for said material and contains tannic acid in such quantity and concentration as to materially 40 exceed that required for mordanting, and subsequently treating with a solution comprising tartar emetic.

45

16. A process for the weighting of material comprising an organic ester of cellulose, 50 which comprises treating said material at about 45° to 80° C. with a solution which is a swelling agent for said material and contains tannic acid in such quantity and concentration as to materially exceed that required for mordanting. 55

17. A process for the weighting of material comprising an organic ester of cellulose, which comprises treating said material at about 45° to 80° C. with a solution which is  
60 a swelling agent for said material and contains tannic acid in such quantity and concentration as to materially exceed that required for mordanting, and with another substance adapted to fix the tannic acid.

**65** 18. A process for the weighting of material

comprising an organic ester of cellulose, which comprises treating said material at about 45° to 80° C. with a solution which is a swelling agent for said material and contains tannic acid in such quantity and concentration as to materially exceed that required for mordanting, and with a solution comprising a metal salt adapted to fix the tannic acid.

19. A process for the weighting of material comprising an organic ester of cellulose, which comprises treating said material at about 45° to 80° C. with a solution which is a swelling agent for said material and contains tannic acid in such quantity and concentration as to materially exceed that required for mordanting, and subsequently treating with a solution comprising a metal salt adapted to fix the tannic acid. 75  
80

20. A process for the weighting of material comprising an organic ester of cellulose, which comprises treating said material at about 45°-80° C. with a solution which is a swelling agent for said material and contains tannic acid in such quantity and concentration as to materially exceed that required for mordanting, and subsequently treating with a solution comprising tartar 85  
90

emetic. 21. A process for the weighting of material 95 comprising cellulose acetate, which comprises treating said material with a solution which is a swelling agent for said material and contains tannic acid in such quantity and concentration as to materially exceed that required 100 for mordanting.

22. A process for the weighting of material comprising cellulose acetate, which comprises treating said material with a solution which is a swelling agent for said material and contains tannic acid in such quantity and concentration as to materially exceed that required for mordanting, and with another substance adapted to fix the tannic acid. 105

23. A process for the weighting of material comprising cellulose acetate, which comprises treating said material with a solution which is a swelling agent for said material and contains tannic acid in such quantity and concentration as to materially exceed that required for mordanting, and with a solution comprising a metal salt adapted to fix the tannic acid. 110 115

24. A process for the weighting of material comprising cellulose acetate, which comprises treating said material with a solution which is a swelling agent for said material and contains tannic acid in such quantity and concentration as to materially exceed that required for mordanting, and subsequently treating with a solution comprising a metal salt adapted to fix the tannic acid. 120 125

25. A process for the weighting of material comprising cellulose acetate, which comprises treating said material with a solution 130

which is a swelling agent for said material and contains tannic acid in such quantity and concentration as to materially exceed that required for mordanting, and subsequently 5 treating with a solution comprising tartar emetic.

26. A process for the weighting of material comprising cellulose acetate, which comprises treating said material at about 45° to 10 80° C. with a solution which is a swelling agent for said material and contains tannic acid in such quantity and concentration as to materially exceed that required for mordanting.

15 27. A process for the weighting of material comprising cellulose acetate, which comprises treating said material at about 45° to 20 80° C. with a solution which is a swelling agent for said material and contains tannic acid in such quantity and concentration as to materially exceed that required for mordanting, and with another substance adapted to fix the tannic acid.

28. A process for the weighting of material comprising cellulose acetate, which comprises treating said material at about 45° to 25 80° C. with a solution which is a swelling agent for said material and contains tannic acid in such quantity and concentration as to 30 materially exceed that required for mordanting, and with a solution comprising a metal salt adapted to fix the tannic acid.

29. A process for the weighting of material comprising cellulose acetate, which comprises treating said material at about 45° to 35 80° C. with a solution which is a swelling agent for said material and contains tannic acid in such quantity and concentration as to materially exceed that required for mordanting, and subsequently treating with a solution 40 comprising a metal salt adapted to fix the tannic acid.

30. A process for the weighting of material comprising cellulose acetate, which comprises treating said material at about 45° to 45 80° C. with a solution which is a swelling agent for said material and contains tannic acid in such quantity and concentration as to materially exceed that required for mordanting, and subsequently treating with a solution 50 comprising tartar emetic.

In testimony whereof, we have hereunto subscribed our names.

CAMILLE DREYFUS.  
HERBERT PLATT.